

## UNITED STATES PATENT OFFICE

2,419,584

## MINERAL OIL COMPOSITION

Thomas T. Noland, Richmond, Ky., assignor to  
Socony-Vacuum Oil Company, Incorporated, a  
corporation of New York

No Drawing. Application January 18, 1945,  
Serial No. 573,466

12 Claims. (Cl. 252—46.6)

1

This invention has to do with the stabilization of viscous mineral oil fractions against the deleterious effects of oxidation or deterioration with use by the addition thereto of oxidation-inhibitors. More specifically, the invention is directed to the improvement of viscous mineral oil fractions by a combination of such inhibitors; namely, a primary oxidation inhibitor and a secondary inhibitor which when admixed with a viscous mineral oil in minor proportions will prevent or delay certain other undesirable changes taking place in the oil.

As is well known to those familiar with the art, substantially all of the numerous fractions obtained from mineral oils and refined for their various uses are susceptible to oxidation. The susceptibility of an oil fraction to oxidation and the manner in which such oxidation manifests itself within the oil varies with the type and degree of refinement to which the oil has been subjected and with the conditions under which it is used or tested; that is, the products formed in an oil fraction as a result of oxidation and the degree to which they are formed depends upon the extent to which the various unstable constituents or constituents which may act as oxidation catalysts have been removed by refining operations and also upon the conditions of use to which the oil is put.

The present invention is predicated upon the discovery that the oxidation characteristics of viscous mineral oil fractions are greatly improved by the incorporation therein of minor proportions of each of two inhibitors which are designated herein as primary oxidation inhibitors and secondary inhibitors.

The primary oxidation inhibitors contemplated herein are stable, oil-soluble phosphorus- and sulfur-containing reaction products obtained by reaction of phosphorus penta-sulfide and a cycle stock characterized by an olefin and an aromatic content of from about 3 per cent to about 7 per cent and from about 40 per cent to about 60 per cent, respectively, under the following interrelated reaction conditions:

1. Between about 1 per cent and about 8 per cent by weight of  $P_2S_5$  based upon the weight of said cycle stock,

2. A temperature between about  $125^{\circ}$  C. and about  $200^{\circ}$  C., and

3. A relatively short reaction time.

The hydrocarbon reactants are, as indicated above, cycle stocks containing from about 3 per cent to about 7 per cent of olefins and from about

2

40 per cent to about 60 per cent of aromatics, as determined by the following test method:

Twenty-five milliliters of a solution containing 70 per cent by weight of sulfuric acid (sp. gr. 1.84) and 30 per cent of  $P_2O_5$  are placed in a glass stoppered sulfonation bottle (a modified Babcock bottle—A. S. T. M. Standards on Petroleum Products and Lubricants, Sept. 1943, page 381). The bottle is immersed in ice water for five minutes; then 10 milliliters of the hydrocarbon are added. The bottle is shaken for 10 minutes while cooling with ice water. Sulfuric acid (sp. gr. 1.84) is added until the top meniscus of the hydrocarbon layer is brought up to the 100 per cent mark on the graduated portion of the neck. The bottle is then stoppered and is centrifuged for 10 minutes. The milliliters of hydrocarbon oil layer remaining are read and this value is subtracted from the original 10 milliliters to obtain the combined amounts of aromatic and olefin contents of the sample. By repeating the same procedure, except for using 85 per cent sulfuric acid instead of the  $H_2SO_4-P_2O_5$  mixture, the olefinic content of the sample is obtained. Thus olefinic content subtracted from the combined olefin and aromatic content gives the amount of aromatic material present.

Preferably, the hydrocarbon reactants are also characterized by the following: boiling range from about  $90^{\circ}$  C. to about  $400^{\circ}$  C., and specific gravity from about 0.88 to about 0.93. In general, such cycle stocks are obtained from thermal cracking operations of crude oils, but other stocks characterized as above may also be used. Typical of such other stocks are light gas oils, such as a light gas oil containing 4 per cent olefins and 46 per cent aromatics, a specific gravity of 0.8833 and a boiling range from  $150^{\circ}$  C. to  $380^{\circ}$  C. For this reason, the hydrocarbon reactants may be broadly considered as hydrocarbon stocks characterized by the aforesaid percentages of olefins and aromatics.

The amount of  $P_2S_5$  reacted with the cycle stocks contemplated herein is an important consideration. Stable, oil-soluble reaction products containing appreciable quantities of phosphorus and sulfur are obtained when the amount of  $P_2S_5$  so reacted is from about 1 per cent to about 8 per cent by weight of the hydrocarbon reactant. Particularly preferred reaction products, however, are obtained with about 5 per cent by weight of  $P_2S_5$ . When amounts of the order of 10 per cent and 15 per cent of  $P_2S_5$  are used, it has been found that the phosphorus- and sulfur-containing reaction products obtained therewith are un-

stable when heated and are oil-insoluble. As used herein the term "oil soluble" is descriptive of those reaction products which are soluble in oil in amounts of at least 1 per cent by weight.

Another important consideration in the preparation of the aforesaid reaction products is reaction time. In general, superior reaction products, in quantities such as shown in the following examples, are obtained when the reaction time is relatively short, such as from about 2 hours to about 8 hours. While reaction times as long as about 12 hours have been used and satisfactory reaction products obtained therewith, reaction times in the neighborhood of 4 hours are preferred. It is to be understood, however, that the reaction time may be varied considerably depending upon the quantities of reactants and the reaction temperatures used in the preparation of said reaction products.

The interrelation of the foregoing reaction factors will be apparent from the following typical examples recited below, and also those set forth in Table I.

#### EXAMPLE 1

A reaction stock—recycle stock A—from a ther-

product—product B—contained 1.26 per cent phosphorus and 3.6 per cent sulfur.

#### EXAMPLE 3

Five hundred grams of product B obtained in Example 2 were vacuum distilled to a maximum temperature of 172° C. at 3 mm. in order to remove unreacted recycle stock therefrom. The residue—product C—contained 3.34 per cent phosphorus and 7.9 per cent sulfur.

Reaction products obtained from recycle stock A and prepared as in Example 2 above are shown in Table I below in order to demonstrate the influence of each of the several reaction variables—time, temperature and concentration of  $P_2S_5$ . The copper strip tests referred to in the table were made by immersing a polished copper strip in a 1 per cent blend of a reaction product in oil and heating the blend at 100° C. for 24 hours. The copper strip test indicates the presence or absence of free or active sulfur which corrodes copper. An asterisk (\*) has been used in the table wherever the copper strip used in the copper strip test was not corroded in each test; that the reaction product was stable; and that the reaction product was soluble in oil.

Table I

| Product             | Percent $P_2S_5$ (by wt.) | Temp., °C. | Time, Hrs. | Composition |           | Copper Strip Test | Stability | Solubility |
|---------------------|---------------------------|------------|------------|-------------|-----------|-------------------|-----------|------------|
|                     |                           |            |            | Percent P   | Percent S |                   |           |            |
| Temp.:              |                           |            |            |             |           |                   |           |            |
| D                   | 5                         | 150        | 4          | 1.41        | 3.4       | :                 | :         | :          |
| E                   | 5                         | 190-200    | 4          | 1.23        | 3.8       | :                 | :         |            |
| F                   | 5                         | 220        | 4          |             |           |                   | Unstable  | Insoluble. |
| Time:               |                           |            |            |             |           |                   |           |            |
| D                   | 5                         | 150        | 4          | 1.41        | 3.4       | :                 | :         | :          |
| G                   | 5                         | 150        | 8          | 1.26        | 3.6       | :                 | :         | :          |
| H                   | 5                         | 150        | 12         | 1.2         | 3.4       | :                 | :         | :          |
| Cone. of $P_2S_5$ : |                           |            |            |             |           |                   |           |            |
| I                   | 2.3                       | 150        | 4          | 0.62        | 1.89      | :                 | :         | :          |
| D                   | 5                         | 150        | 4          | 1.41        | 3.4       | :                 | :         | :          |

mal liquid phase cracking operation and having the following characteristics, was used:

|                      |          |        |
|----------------------|----------|--------|
| Olefin content       | per cent | 6      |
| Aromatic content     | do       | 47     |
| Specific gravity     |          | 0.8939 |
| Aniline number       |          | 105.5  |
| Boiling range (°C.): |          |        |
| Initial B. Pt        |          | 97     |
| 10                   | per cent | 230    |
| 50                   | do       | 274    |
| 90                   | do       | 327    |
| End point            |          | 366    |
| Recovery             | per cent | 98.5   |

One thousand grams of recycle stock A was reacted, with stirring, with 70 grams of  $P_2S_5$  at 180° C. for 8 hours. The reaction mixture thus obtained was diluted with naphtha (boiling range 88-135° C.), washed with 20 per cent  $Na_2S$  solution, water washed, filtered and the filtrate heated to 150° C. at 10 min. pressure to remove the naphtha. The reaction product contained 1.19 per cent phosphorus and 3.06 per cent sulfur, and is identified hereinafter as product A.

#### EXAMPLE 2

One thousand grams of recycle stock A was reacted, with stirring, with 50 grams of  $P_2S_5$  at 150° C. for 8 hours. The reaction mixture so obtained was then cooled to 100° C., 52.5 grams (5 per cent by weight) of *Attapulgus* clay was added thereto and the clay was subsequently removed therefrom by filtering. The reaction prod-

It will be apparent from the data tabulated in Table I above that reaction temperatures in excess of 200° C. are unsatisfactory. The desired reaction products as indicated in Table I are those prepared under the reaction conditions defined hereinabove.

Another cycle stock which was also found to be particularly desirable was a cycle stock, obtained from a Cross still, and characterized by the following:

|                  |          |        |
|------------------|----------|--------|
| Olefin content   | per cent | 5      |
| Aromatic content | do       | 57     |
| Specific gravity |          | 0.9236 |
| Aniline number   |          | 80     |

Boiling range °C. 140-370

While products A, B and C, shown above in Examples 1 through 3, and products D, E, G, H and I shown in Table I are particularly desirable for use in petroleum fractions, related reaction products prepared in a similar manner from other hydrocarbon reactants are undesirable for such use. The data presented in Table II below is illustrative of their undesirable character. The copper strip tests referred to in this table were obtained in the manner described in connection with Table I. The heat stability tests shown in Table II were made by heating a 1 per cent blend of a reaction product in oil at 100° C. for 24 hours. An asterisk has been used as in Table I to indicate that the copper strip in the copper strip tests was not corroded in each test, and that the reaction product was stable to heat.

Table II

| Hydrocarbon                                                                                    | Prod-<br>uct | Per cent<br>P <sub>2</sub> S <sub>5</sub><br>(by wt.) | Temp.,<br>° C. | Temp.,<br>hours | Composi-<br>tion |                  | Copper Strip<br>test  | Heat<br>Stability     | Remarks                                                                               |
|------------------------------------------------------------------------------------------------|--------------|-------------------------------------------------------|----------------|-----------------|------------------|------------------|-----------------------|-----------------------|---------------------------------------------------------------------------------------|
|                                                                                                |              |                                                       |                |                 | Per<br>cent<br>P | Per<br>cent<br>S |                       |                       |                                                                                       |
| Catalytically Cracked Cycle Stock:<br>Percent Olefin, 3<br>Percent Aromatic, 35                | M            | 5                                                     | 190-195        | 4½              | 0.88             | 2.1              | Corrosive black strip | Poor sludge deposited | Sludge formed during reaction; additional oil-insoluble sludge separated on standing. |
| Catalytically Cracked Cycle Stock:<br>Percent Olefin, 1<br>Percent Aromatic, 35                | N            | 5                                                     | 190-195        | 4½              | 1.04             | 2.0              | do                    | do                    | Do.                                                                                   |
| No. 2 Fuel Oil from Catalytic Cracking Operation:<br>Percent Olefin, 0<br>Percent Aromatic, 36 | O            | 5                                                     | 180-200        | 2½              | do               | do               | Unstable              | do                    | Do.                                                                                   |

It will be apparent from the results set forth in Table II above that the reaction products of hydrocarbon reactants which are not characterized by the required olefin and aromatic contents defined above are greatly inferior to the related reaction products from the cycle stocks contemplated herein and illustrated in Examples 1 through 3 and in Table I. For example, it is apparent that the reaction products obtained from the catalytic cycle stocks and the No. 2 fuel oil defined in Table II are corrosive to copper and are unstable when heated, being so unstable when heated that considerable quantities of oil insoluble sludge are deposited therefrom. Thus, the latter reaction products have little or no value as addition agents for petroleum fractions, particularly viscous mineral oils. On the contrary, however, the reaction products contemplated herein are not corrosive to copper and are stable when heated. It will be recognized, therefore, that the reaction products of this invention are much more marketable in the oil industry and other industries than are the related reaction products of such hydrocarbon reactants as those shown above in Table II.

When used in viscous mineral oil fractions in small amounts, the aforesaid primary oxidation inhibitors effect improvement of several of the oxidation characteristics thereof by preventing, for example, corrosion of hard metal bearings, by inhibition of acid-formation, by inhibition of formation of gummy deposits in engines, by preventing increase in viscosity, etc. However on standing for several days or when heated and then left to stand, an oil composition comprised only of a viscous mineral oil fraction and a primary oxidation inhibitor tends to become cloudy. This shortcoming has now been overcome by incorporating in such oil composition a small amount of a secondary inhibitor.

The secondary inhibitors of this invention which are capable of regulating or preventing the aforesaid haze problem are oil-miscible metal salts of sulfonic acids. These sulfonic acids include both those prepared from aromatic hydrocarbons, or substituted aromatic hydrocarbons, by treatment with strong sulfuric acid, oleum, chlorsulfonic acid, etc., and those obtained by treatment of various petroleum fractions with the same reagents. Any metallic salt of any organic sulfonic acid that is sufficiently soluble in petroleum oils is contemplated by this invention as the secondary inhibitor. Among the metals which are especially suitable for this purpose are sodium, potassium, magnesium, calcium, cobalt, tin, strontium and barium. Particularly preferred are barium, sodium and calcium.

Of the sulfonic acids contemplated by the present invention, preference is given to the substituted aromatic sulfonic acids and to the petroleum sulfonic acids. Both mono- and poly-substituted aromatic sulfonic acids are contemplated, particular preference being given to the alkyl-substituted benzene sulfonic acids. Of the mono- and poly-alkyl substituents for the aromatic sulfonic acids, the so-called "wax" substituents—that is, those alkyl substituents containing at least about 20 carbon atoms—are particularly preferred.

The particularly-preferred compositions of primary and secondary inhibitors in viscous mineral oil fractions which are contemplated herein are those in which the primary inhibitor is a P<sub>2</sub>S<sub>5</sub>-cycle stock reaction product or a P<sub>2</sub>S<sub>5</sub>-light gas

oil reaction product, of the type described above, and the secondary inhibitor is either barium or calcium diwax benzene sulfonate, barium or calcium petroleum sulfonate, or sodium petroleum sulfonate.

As stated above, oil compositions comprising only a viscous mineral oil fraction and a typical primary oxidation inhibitor have a tendency to develop a haze, the formation of which can be suppressed by the addition to such compositions of a small amount of a secondary inhibitor, namely, an oil-miscible metal salt of a sulfonic acid. This fact is demonstrated by the test results set forth in table III below. The oil used in these tests was a solvent-refined S. A. E. 10 grade motor oil.

The P<sub>2</sub>S<sub>5</sub>-cycle stock reaction product (product B) was prepared as described in Example 2 above.

The barium diwax benzene sulfonate used as the haze-inhibitor was prepared by reacting a 10 per cent chlor-paraffin wax with benzene to form a diwax benzene, which was treated with oleum to form the sulfonic acid, which in turn was neutralized with barium hydroxide. In order to reduce the viscosity and to increase the ease of handling, this product was blended in a 1:1 ratio with an S. A. E. 30 grade motor oil. The blend contained 5.17 per cent barium and 1.5 per cent sulfur.

The sodium petroleum sulfonate used in these tests was the sodium salt of an oil-soluble sulfonic acid prepared by treating a Mid-Continent distillate of 95 seconds Saybolt Universal viscosity at 100° F. with oleum. It contained 2.57 per cent sulfur.

The barium petroleum sulfonate was prepared from the above sodium salt by treatment with BaCl<sub>2</sub> solution. It contained 6.9 per cent barium.

The various blends indicated in Table III were placed in 4-ounce bottles and kept at room tem-

perature in diffused light for the length of time given below, with the following results:

soluble, phosphorus- and sulfur-containing reaction product obtained by reaction of phos-

Table III

| Primary Inhibitor | Conc., Wt. Per Cent | Secondary Inhibitor             | Conc., Wt. Per Cent | Appearance                          |
|-------------------|---------------------|---------------------------------|---------------------|-------------------------------------|
| Product B         | 3                   |                                 |                     |                                     |
| Do.               | 3                   | Barium diwax benzene sulfonate. | 0.3                 | Haze in 1 day.<br>Clear at 30 days. |
| Do.               | 3                   | Barium petroleum sulfonate.     | 0.3                 | Do.                                 |
| Do.               | 3                   | Sodium petroleum sulfonate.     | 0.3                 | Do.                                 |

The results shown above in Table III demonstrate effectively that haze-formation in an oil containing as a primary oxidation inhibitor a  $P_2S_5$ -cycle stock reaction product is appreciably inhibited by the addition of a small amount of 20 the secondary inhibitor contemplated by this invention.

The amount of secondary inhibitor necessary to effect the desired haze-inhibition depends upon the concentration of primary oxidation inhibitor in the oil as well as upon the type of mineral oil fraction used. In general, however, from about 1.0 to about 10.0 per cent by weight of the secondary inhibitor based upon the amount of primary inhibitor present will be sufficient to effectively regulate haze-formation. The amount of primary oxidation inhibitor contemplated for use in the oil compositions of the present invention is from about 0.1 per cent to about 3.0 per cent, although about 0.1 per cent to about 1 per cent of these reaction products will usually suffice. Accordingly, the amount of secondary inhibitor used in the oil blend will be from about 0.001 per cent to about 0.3 per cent by weight.

As contemplated herein, the primary and secondary inhibitors of this invention may be incorporated in a viscous mineral oil fraction either by adding the secondary inhibitor to the primary inhibitor before both are blended with the oil or by adding the secondary inhibitor separately to the blend of the oil and the primary inhibitor. The term, "mineral oil composition," as used herein and as recited in all of the appended claims, is inclusive of all mineral oil fractions containing a primary oxidation inhibitor and a secondary inhibitor and of all oil compositions obtained or prepared by any of the procedures hereinabove described. Any oil compositions so obtained or prepared is substantially free of haze normally occurring in an oil composition containing the primary oxidation inhibitor alone.

It is also to be understood that the examples, procedures, and oil compositions described herein are illustrative only and are not to be construed as limiting the scope of this invention thereto. Thus, all cycle stocks and light gas oils as defined above may be used in place of those shown in the foregoing examples; any metallic salt of any sulfonic acid that is sufficiently soluble in petroleum oils is suitable for use as the secondary inhibitor; and the mineral oils disclosed above are but typical of all viscous mineral oil fractions which may be used in this invention.

I claim:

1. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-

phorus penta-sulfide and a hydrocarbon stock at a temperature between about 125° C. and about 200° C. for a relatively short reaction time, said hydrocarbon stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending to form a haze in the oil; and a minor proportion, from about 0.001 per cent to about 0.3 per cent, sufficient to suppress the formation of said haze, of an oil-miscible metal salt of a sulfonic acid.

2. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a light gas oil at a temperature between about 125° C. and about 200° C. for a relatively short reaction time, said light gas oil being characterized by an olefin content of about 4 per cent and an aromatic content of about 46 per cent, said phosphorus penta-sulfide representing about 5 per cent by weight of said light gas oil, and the said reaction product normally tending to form a haze in the oil; and a minor proportion, from about 0.001 per cent to about 0.3 per cent, sufficient to suppress the formation of said haze, of an oil-miscible metal salt of a sulfonic acid.

3. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a cycle stock at a temperature between about 125° C. and about 200° C. for a relatively short reaction time, said cycle stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible metal salt of a sulfonic acid.

4. A mineral oil composition comprising a viscous mineral oil fraction containing a minor proportion, from about 0.1 per cent to about 3.0 per cent, sufficient to inhibit the deteriorating

effects of oxidation upon the oil, of a stable, oil-soluble, phosphorus- and sulfur-containing reaction product obtained by reaction of phosphorus penta-sulfide and a cycle stock at a temperature between about 125° C. and about 200° C. for a reaction time from about 2 hours to about 8 hours, said cycle stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible metal salt of a sulfonic acid.

5. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a cycle stock at about 150° C. for about 8 hours, said cycle stock being characterized by an olefin content of about 6 per cent and an aromatic content of about 47 per cent, said phosphorus penta-sulfide representing about 5 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible metal salt of a sulfonic acid.

6. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble phosphorus- and sulfur-containing reaction product obtained by reaction of phosphorus penta-sulfide and a hydrocarbon stock at a temperature between about 125° C. and about 200° C. for a relatively short reaction time, said hydrocarbon stock being characterized by an olefinic content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending to form a haze in the oil; and a minor proportion, from about 0.001 per cent to about 0.3 per cent, sufficient to suppress the formation of said haze, of an oil-miscible metal salt of an alkyl-substituted aromatic sulfonic acid.

7. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a hydrocarbon stock at a temperature between about 125° C. and about 200° C. for a relatively short reaction time, said hydrocarbon stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending

to form a haze in the oil; and a minor proportion, from about 0.001 per cent to about 0.3 per cent, sufficient to suppress the formation of said haze, of an oil-miscible metal salt of an alkyl-substituted benzene sulfonic acid.

8. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a hydrocarbon stock at a temperature between about 125° C. and about 200° C. for a relatively short reaction time, said hydrocarbon being characterized by an olefin content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending to form a haze in the oil; and a minor proportion, from about 0.001 per cent to about 0.3 per cent, sufficient to suppress the formation of said haze, of an oil-miscible metal salt of a wax-substituted benzene sulfonic acid.

9. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a hydrocarbon stock at a temperature between about 125° C. and about 200° C. for a relatively short reaction time, said hydrocarbon stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending to form a haze in the oil; and a minor proportion, from about 0.001 per cent to about 0.3 per cent, sufficient to suppress the formation of said haze, of an oil-miscible barium salt of diwax-substituted benzene sulfonic acid.

10. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus-penta-sulfide and a hydrocarbon stock at a temperature between about 125° C. and about 200° C. for a relatively short reaction time, said hydrocarbon stock being characterized by an olefin content of from about 3 per cent to about 7 per cent and an aromatic content of from about 40 per cent to about 60 per cent, said phosphorus penta-sulfide representing from about 1 per cent to about 8 per cent by weight of the said hydrocarbon stock, and the said reaction product normally tending to form a haze in the oil; and a minor proportion, from about 0.001 per cent to about 0.3 per cent, sufficient to suppress the formation of said haze, of an oil-miscible metal salt of a petroleum sulfonic acid.

11. A mineral oil composition comprising a viscous mineral oil fraction containing a minor proportion, from about 0.1 per cent to about 3.0 per cent, sufficient to inhibit the deteriorating effects

of oxidation upon the oil, of a stable, oil-soluble, phosphorus- and sulfur-containing reaction product obtained by reaction of phosphorus penta-sulfide and a cycle stock at about 150° C. for about 8 hours, said cycle stock being characterized by an olefin content of about 6 per cent and an aromatic content of about 47 per cent, said phosphorus penta-sulfide representing about 5 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible barium salt of diwax-substituted benzene sulfonic acid.

12. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a cycle stock at about 150° C. for about 8 hours, said cycle stock being characterized by an olefin content of about 6 per cent

10

15

20

25

and an aromatic content of about 47 per cent, said phosphorus penta-sulfide representing about 5 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible sodium salt of a petroleum sulfonic acid.

THOMAS T. NOLAND.

## REFERENCES CITED

The following references are of record in the file of this patent:

## UNITED STATES PATENTS

| Number    | Name      | Date          |
|-----------|-----------|---------------|
| 2,136,391 | Miller    | Nov. 15, 1938 |
| 2,202,394 | Morway    | May 28, 1940  |
| 2,279,086 | Bergstrom | Apr. 7, 1942  |
| 2,315,529 | Kelso     | Apr. 6, 1943  |
| 2,316,082 | Loane     | Apr. 6, 1943  |
| 2,342,572 | Cook      | Feb. 22, 1944 |
| 2,365,209 | Musselman | Dec. 19, 1944 |
| 2,373,094 | Berger    | Apr. 10, 1945 |

## Certificate of Correction

Patent No. 2,419,584.

April 29, 1947.

THOMAS T. NOLAND

It is hereby certified that error appears in the printed specification of the above numbered patent requiring correction as follows: Column 6, Table II, under the heading "Copper Strip test" strike out the last "do"; and that the said Letters Patent should be read with this correction therein that the same may conform to the record of the case in the Patent Office.

Signed and sealed this 29th day of July, A. D. 1947.

[SEAL]

LESLIE FRAZER,  
*First Assistant Commissioner of Patents.*

of oxidation upon the oil, of a stable, oil-soluble, phosphorus- and sulfur-containing reaction product obtained by reaction of phosphorus penta-sulfide and a cycle stock at about 150° C. for about 8 hours, said cycle stock being characterized by an olefin content of about 6 per cent and an aromatic content of about 47 per cent, said phosphorus penta-sulfide representing about 5 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible barium salt of diwax-substituted benzene sulfonic acid.

12. A mineral oil composition comprising a viscous mineral oil fraction containing a minor proportion, from about 0.1 per cent to about 3.0 per cent, sufficient to inhibit the deteriorating effects of oxidation upon the oil, of a stable, oil-soluble, phosphorus- and sulfur-containing reaction product obtained by reaction of phosphorus penta-sulfide and a cycle stock at about 150° C. for about 8 hours, said cycle stock being characterized by an olefin content of about 6 per cent

10

15

20

25

and an aromatic content of about 47 per cent, said phosphorus penta-sulfide representing about 5 per cent by weight of the said cycle stock, and the said reaction product normally tending to form a haze in the oil; and a minor proportion, from about 0.001 per cent to about 0.3 per cent, sufficient to suppress the formation of said haze, of an oil-miscible sodium salt of a petroleum sulfonic acid.

THOMAS T. NOLAND.

## REFERENCES CITED

The following references are of record in the file of this patent:

## UNITED STATES PATENTS

| Number    | Name      | Date          |
|-----------|-----------|---------------|
| 2,136,391 | Miller    | Nov. 15, 1938 |
| 2,202,394 | Morway    | May 28, 1940  |
| 2,279,086 | Bergstrom | Apr. 7, 1942  |
| 2,315,529 | Kelso     | Apr. 6, 1943  |
| 2,316,082 | Loane     | Apr. 6, 1943  |
| 2,342,572 | Cook      | Feb. 22, 1944 |
| 2,365,209 | Musselman | Dec. 19, 1944 |
| 2,373,094 | Berger    | Apr. 10, 1945 |

## Certificate of Correction

Patent No. 2,419,584.

April 29, 1947.

THOMAS T. NOLAND

It is hereby certified that error appears in the printed specification of the above numbered patent requiring correction as follows: Column 6, Table II, under the heading "Copper Strip test" strike out the last "do"; and that the said Letters Patent should be read with this correction therein that the same may conform to the record of the case in the Patent Office.

Signed and sealed this 29th day of July, A. D. 1947.

[SEAL]

LESLIE FRAZER,  
*First Assistant Commissioner of Patents.*